# EUROPEAN PATENT SPECIFICATION

(11) **EP 1 726 685 B1**
(45) Date of publication and mention of the grant of the patent: **11.07.2012**
(21) Application number: 06252535.7
(22) Date of filing: 15.05.2006
(51) Int. Cl.: C23C 28/00, C23C 14/30

(54) **Manufacturing method of a thermal barrier coating**
Herstellungsverfahren einer Wärmedämmschicht
Procédé de fabrication d'un revêtement de barrière thermique

(30) Priority: 27.05.2005 SG 200503371
(43) Date of publication of application: 29.11.2006
(73) Proprietor: Turbine Overhaul Services Private Limited, Singapore 638639 (SG)
(72) Inventor: Luah, Kok Hai, Singapore 640 552 (SG); Rao, Garimella B., Singapore 669 618 (SG)
(74) Representative: Leckey, David Herbert

(56) References cited:
- EP-A- 0 267 143
- EP-A- 1 522 608
- US-A1- 2002 055 004
- US-A1- 2003 224 200

## Description

### BACKGROUND OF THE INVENTION

This invention relates to thermal barrier coatings, and more particularly to bond coats for thermal barrier coatings on turbine components.

Gas turbine engine components (e.g., blades, vanes, seals, combustor panels, and the like) are commonly formed of nickel- or cobalt based superalloys. Desired operating temperatures often exceed that possible for the alloys alone. Thermal barrier coatings (TBCs) are in common use on such components to permit use at elevated temperatures. Various coating compositions (e.g., ceramics) and various coating methods (e.g., electron beam physical vapor deposition (EB-PVD) and plasma spray deposition) are known.

An exemplary modern coating system is applied to the superalloy substrate by an EB-PVD technique. An exemplary coating system includes a metallic bondcoat layer (e.g., an overlay of NiCoCrAlY alloy or diffusion aluminide) atop the substrate. A thermally insulating ceramic topcoat layer (e.g., zirconia stabilized with yttria (YSZ)) is deposited atop the bondcoat. During this deposition, a thermally grown oxide layer (TGO) (e.g., alumina) may form on the bondcoat and intervenes between the remaining underlying portion of the bondcoat and the topcoat.

In one exemplary coating system e.g. in US 2002/0055004 A, a nickel-based superalloy substrate is initially plated with platinum. Thereafter, a coating of aluminum is applied. During the aluminum application diffusion may form a platinum-containing aluminide. After this coating, a further heating step causes further diffusion resulting in greater uniformity by diffusing in excess surface aluminum and diffusing out nickel from the substrate. Thereafter, the YSZ coating is deposited by EB-PVD.

A prior art method of coating an article, having the features of the preamble of claim 1 is disclosed in US 2002/0055004. Another prior art method is disclosed in "Improved Oxidation Resistance of Thermal Barrier Coatings" by Kh.G.Schmitt-Thomas, M. Hertter, XP-001 004 807.

### SUMMARY OF THE INVENTION

According to the present invention, there is provided a method as claimed in claim 1.

The method provides a coated article including a substrate and a thermal barrier layer. An aluminide layer is between the substrate and the thermal barrier layer. A PtAl₂ layer is between the aluminide layer and the thermal barrier layer.

The details of one or more embodiments of the invention are set forth in the accompanying drawings and the description below.

### BRIEF DESCRIPTION OF THE DRAWINGS

FIG. 1 is a basic flowchart of a process for forming a coated article.
FIG. 2 is a sectional photomicrograph of a coated article.
FIG. 3 is a flowchart of an alternative process for forming a coated article, that is outside the scope of the present invention.

Like reference numbers and designations in the various drawings indicate like elements.

### DETAILED DESCRIPTION

FIG. 1 shows an exemplary process for forming a coated article. The exemplary process includes forming a substrate to be coated. Exemplary substrates are gas turbine engine components formed of nickel- or cobalt- based superalloys. One component of particular interest is a turbine section blade. The substrate may be formed by one or more steps (e.g., casting and machining). Alternatively, in a re-coating situation the substrate may have previously been formed and may be subject to removal of an existing coating and optional patching, crack filling, and the like.

The surface of the substrate to be coated may be prepared by chemical and/or mechanical means (e.g., cosmetic blasting as is known in the art). Thereafter, an aluminum-containing material is applied directly to the substrate surface. The application of the aluminum-containing material will serve to at least initially form an aluminide. Many application techniques are used in the art and are possible. An exemplary technique involves a conventional gas phase coating. Such a process involves placing the substrate in proximity to a coating media source generating coating vapors. This may be distinguished from chemical vapor deposition (CVD) techniques wherein the source is more remote. In CVD coating, the substrate is kept in a container which is separate from the coating media container(s). The CVD coating material vapors are delivered via separate carrier gas. In gas phase coating the substrate and the coating media are in the same container and the substrate does not touch the coating media (from which the coating vapors are generated).

An exemplary source material comprises aluminum chrome with ammonium fluoride, ammonium chloride, or aluminum flouride as an activator. Exemplary aluminum chrome is a granular alloy of aluminum and chromium in a eutectic 55:45 weight percent ratio. Upon heating of the aluminum chrome and activator (e.g., in a pan under controlled atmosphere conditions such as an inert gas(e.g., argon)), the activator causes release of an aluminum vapor which condenses on the substrate. An exemplary deposition duration is less than eight hours (e.g., five to seven hours) .During this deposition, diffusion from the substrate (e.g., especially of nickel) converts the applied aluminum-containing material into nickel aluminide. This aluminide will tend to have an NiAl/NiAl₂ composition further including other of the substrate alloying elements as alloying elements in the aluminide and/or as precipitates in the aluminide.

After the application of the aluminum-containing material and initial aluminide formation, a platinum-containing material is applied. The exemplary application involves electroplating of pure platinum. This application leaves a layer of the platinum-containing material atop the aluminide.

A diffusion step then produces diffusion of aluminum into the platinum layer and of platinum into the aluminide. An exemplary diffusion is caused by heating. Exemplary heating is to a temperature of at least 1850°F (1010°C) (more preferably at least 1900°F (1038°C), more preferably still, 1950°F (1065°C)) for a time of at least five minutes (e.g., to about 1925°F (1052°C) for about ten minutes in vacuum (e.g., 0.1 militorr or less) then 1975°F (1079°C) for about four hours in argon).

After any additional surface preparation (e.g., polishing) the YSZ coating may be applied. An exemplary YSZ application is by EB-PVD.

FIG. 2 shows details of the coated article. The substrate has a largely undisturbed base portion 20 at the bottom of the figure. The YSZ layer 22 is at the top. The YSZ layer 22 is immediately atop a platinum-aluminum layer 24 produced by the diffusion of aluminum into the platinum plating. In an exemplary implementation, the layer 24 is a continuous PtAl₂ phase. The platinum-containing aluminide layer 26 is below the PtAl₂ layer 24. A transition region 30 between the layers 24 and 26 is not extremely abrupt and is characterized by moderately large inclusions of one layer's material within the other. The transition region 30 is located outboard of the original boundary between the aluminide and the platinum plating. This boundary is evidenced by the dark spots which may be coincident with the original surface of the substrate. Similarly, a diffusion region 28 may be between the undisturbed substrate base portion 20 and the aluminide 26.

An exemplary thickness of the YSZ layer 22 is at least 40µm (e.g., 50-100µm). An exemplary thickness of the PtAl₂ layer 24 is 5-20µm. An exemplary thickness of the aluminide layer 26 is 25-100µm.

Plating after the aluminum deposition may have one or more of several advantages. The plating may tend to provide a smooth surface by filling roughness imperfections in the aluminide. Exemplary roughness is 20-40RA after diffusion. The smoothness promotes topcoat adhesion and associated spall resistance.

FIG. 3 shows an alternative process, not according to the present invention, wherein the order of platinum and aluminum application is reversed. As distinguished from one prior art system wherein platinum is applied directly to a substrate, the platinum layer deposited in FIG. 3 is relatively thick (e.g., 5-8µm). Also, there is substantially no separate diffusion step between the platinum application and the aluminum application. The subsequent diffusion heating (e.g., to at least 1850°F (1010°C) (more preferably 1950°F (1065°C)) for at least five minutes) serves to interdiffuse the platinum into the aluminum (forming the surface layer 24) as well as providing the platinum for the aluminide layer. An exemplary heating is to 1975°F (1079°C) for about four hours in argon. The diffusion also passes substrate components (e.g., the nickel) into the aluminum to form the aluminide layer.

## Claims

1. A method **characterised by** the steps of:
applying an aluminum-containing material to a substrate (20), causing diffusion from the substrate (20) into the applied aluminum containing material so as to form an aluminide first layer (26);
applying a platinum-containing second layer (24) atop the aluminide first layer (26);
causing diffusion of aluminum from the aluminide first layer (26) into the second layer (24) so as to produce a PtAl₂ alloy; and
applying a thermal barrier layer (22) atop the PtAl₂ alloy.

2. The method of claim 1, wherein the applying the thermal barrier layer (22) comprises electron beam physical vapor deposition of yttria-stabilized zirconia.

3. The method of claim 1 or 2, wherein the applying the aluminum-containing material consists essentially of gas phase coating of aluminum chrome with an activator.

4. The method of claim 1, 2 or 3, wherein causing diffusion of aluminum into the second layer (24) comprises heating to a temperature of at least 1850°F (1010°C).

5. The method of claim 1, wherein the causing diffusion of aluminum into the second layer (24) comprises heating to a temperature of at least 1900°F (1038°C).

6. The method of claim 1, 2 or 3, wherein the diffusion of aluminum into the second layer (24) is at least as great as a diffusion caused by heating to a temperature of 1850°F (1010°C) for a time of at least five minutes.

7. The method of claim 1, 2 or 3, wherein the diffusion of aluminum into the second layer (24) is at least as great as a diffusion caused by heating to a temperature of 1925°F (1052°C) for a time of at least five minutes.

8. The method of claim 1, 2 or 3, wherein the diffusion of aluminum into the second layer (24) is at least as great as a diffusion caused by heating to a temperature of 1950°F (1079°C) for a time of at least five minutes.

9. The method of any of claims 1 to B, further comprising:
forming the substrate (20) of a nickel-based superalloy.

10. The method of any of claims 1 to 9, further comprising:
preparing the substrate (20) by surface blasting.

## Patentansprüche

1. Verfahren **gekennzeichnet durch** die Schritte:
Aufbringen eines Aluminium enthaltenden Materials auf ein Substrat (20), Verursachen von Diffusion von dem Substrat (20) in das aufgebrachte Aluminium enthaltende Material, um eine erste Aluminidschicht (26) auszubilden;
Aufbringen einer Platin enthaltenden zweiten Schicht (24) oben auf die erste Aluminidschicht (26);
Verursachen von Diffusion von Aluminium von der ersten Aluminidschicht (26) in die zweite Schicht (24), um eine PtAl₂-Legierung zu bilden; und
Aufbringen einer thermischen Sperrschicht (22) oben auf die PtAl₂-Legierung.

2. Verfahren nach Anspruch 1, wobei das Aufbringen der thermischen Sperrschicht (22) physikalisches Elektronenstrahl-Gasabscheiden von Yttriumoxid-stabilisiertem Zirkonoxid umfasst.

3. Verfahren nach Anspruch 1 oder 2, wobei das Aufbringen des Aluminium enthaltenden Materials im Wesentlichen aus Gasphasenbeschichten von Aluminium-Chrom mit einem Aktivator besteht.

4. Verfahren nach Anspruch 1, 2 oder 3, wobei das Verursachen von Diffusion von Aluminium in die zweite Schicht (24) Erwärmen auf eine Temperatur von zumindest 1850 ° F (1010 ° C) umfasst.

5. Verfahren nach Anspruch 1, wobei das Verursachen von Diffusion von Aluminium in die zweite Schicht (24) Erwärmen auf eine Temperatur von zumindest 1900 ° F (1038 ° C) umfasst.

6. Verfahren nach Anspruch 1, 2 oder 3, wobei die Diffusion von Aluminium in die zweite Schicht (24) zumindest so groß ist, wie eine durch das Erwärmen auf eine Temperatur von 1850 ° F (1010 ° C) für eine Zeit von zumindest fünf Minuten verursachte Diffusion.

7. Verfahren nach Anspruch 1, 2 oder 3, wobei die Diffusion von Aluminium in die zweite Schicht (24) zumindest so groß ist wie eine durch das Erwärmen auf eine Temperatur von 1925 ° F (1052 ° C) für eine Zeit von zumindest fünf Minuten verursachte Diffusion.

8. Verfahren nach Anspruch 1, 2 oder 3, wobei die Diffusion von Aluminium in die zweite Schicht (24) zumindest so groß ist wie eine durch Erwärmen auf eine Temperatur von 1950° F (1079 ° C) für eine Zeit von zumindest fünf Minuten verursachte Diffusion.

9. Verfahren nach einem der Ansprüche 1 bis 8, des Weiteren umfassend:
Ausbilden des Substrats (20) aus einer Nickel basierenden Superlegierung.

10. Verfahren nach einem der Ansprüche 1 bis 9, des Weiteren umfassend:
Vorbereiten des Substrats (20) durch Oherflächenstrahlen.

## Revendications

1. Procédé **caractérisé par** les étapes qui consistent à :
appliquer un matériau contenant de l'aluminium sur un substrat (20) et amener une diffusion depuis le substrat (20) jusque dans le matériau contenant de l'aluminium ainsi appliqué, de manière à former une première couche d'aluminure (26),
appliquer au-dessus de la première couche d'aluminure (26) une deuxième couche (24) contenant du platine,
amener la diffusion de l'aluminium de la première couche d'aluminure (26) jusque dans la deuxième couche (24) de manière à produire un alliage de PtAl₂ et
appliquer une couche de barrière thermique (22) au-dessus de l'alliage de PtAl₂.

2. Procédé selon la revendication 1, dans lequel l'application de la couche de barrière thermique (22) comprend le dépôt physique par phase vapeur par faisceau d'électrons d'une zircone stabilisée par yttrie.

3. Procédé selon la revendication 1 ou 2, dans lequel l'application du matériau contenant de l'aluminium consiste essentiellement en un revêtement d'aluminium-chrome appliqué en phase gazeuse avec un activateur.

4. Procédé selon la revendication 1, 2 ou 3, dans lequel l'amenée de la diffusion d'aluminium dans la deuxième couche (24) comprend le chauffage à une température d'au moins 1 010° C (1 850° F).

5. Procédé selon la revendication 1, dans lequel l'amenée de la diffusion d'aluminium dans la deuxième couche (24) comprend le chauffage à une température d'au moins 1 038° C (1 900° F).

6. Procédé selon la revendication 1, 2 ou 3, dans lequel la diffusion de l'aluminium dans la deuxième couche (24) est au moins aussi élevée que la diffusion amenée par le chauffage à une température de 1 010° C (1 850° F) pendant une durée d'au moins 5 minutes.

7. Procédé selon la revendication 1, 2 ou 3, dans lequel la diffusion de l'aluminium dans la deuxième couche (24) est au moins aussi élevée que la diffusion amenée par le chauffage à une température de 1 052° C (1 925° F) pendant une durée d'au moins 5 minutes.

8. Procédé selon la revendication 1, 2 ou 3, dans lequel la diffusion de l'aluminium dans la deuxième couche (24) est au moins aussi élevée que la diffusion amenée par le chauffage à une température de 1 079° C (1 950° F) pendant une durée d'au moins 5 minutes.

9. Procédé selon l'une quelconque des revendications 1 à 8, comprenant en outre l'étape qui consiste à former le substrat (20) d'un superalliage à base de nickel.

10. Procédé selon l'une quelconque des revendications 1 à 9, comprenant en outre la préparation du substrat (20) par sablage de sa surface.
